

# UNITED STATES PATENT OFFICE.

HANS GOLDSCHMIDT AND OTTO WEIL, OF ESSEN-ON-THE-RUHR, GERMANY, ASSIGNEES  
TO TH. GOLDSCHMIDT, OF ESSEN-ON-THE-RUHR, GERMANY, A FIRM.

## METHOD OF MANUFACTURING CALCIUM-SILICON ALLOYS, &c.

938,758.

Specification of Letters Patent.

Patented Nov. 2, 1909.

No Drawing.

Application filed June 29, 1908. Serial No. 440,803.

To all whom it may concern:

Be it known that we, HANS GOLDSCHMIDT and OTTO WEIL, subjects of the King of Prussia, German Emperor, and residents 5 of Essen-on-the-Ruhr, in the Province of the Rhine, German Empire, have jointly invented certain new and useful Improvements in the Method of Manufacturing Calcium-Silicon Alloys Containing a High 10 Percentage of Calcium, of which the following is an exact specification.

Calcium-silicon alloys, which theoretically had been determined by the formula  $CaSi_2$ , have already been manufactured several times 15 by reduction of silica or lime together with carbon in an electric furnace. But on account of the reaction of the carbon there were always obtained alloys containing carbon, which alloys had only a relatively small amount 20 of calcium. The highest amount of calcium in these calcium-silicides obtained by the electric process, is stated to be somewhat more than 20 per cent. (De Chalmot 1896.)

The inventors have recently succeeded 25 (see U. S. applications Ser. No. 428,933 and Ser. No. 417,523) in obtaining a calcium-silicon-alloy containing about one third of calcium and two thirds of silicon by heating a mixture of lime and metallic silicon with 30 an addition of suitable fluxes. Now it has been found that this calcium-silicon-alloy may be changed into an alloy containing much more calcium, by melting it down with iron, whereby the iron, under formation 35 of ferro-silicon, combines with such a quantity of silicon that an alloy will be formed containing about two thirds of calcium and one third of silicon. This alloy is of a less specific weight than the ferro-silicon 40 and the latter sinking down to the bottom and thus may easily be separated.

The process may be carried out in any kind of muffles, muffle-furnaces, or in any kind of furnaces which produce such a temperature that the calcium-silicon will be melted.

Any kind of iron may be employed, such as pig-iron, cast-iron, wrought-iron or steel.

The calcium-silicon-alloy may be melted 50 down with iron (in form of chips, small pieces) under a protecting layer of chlorid of calcium. Or the calcium-silicon-alloy may be melted alone as well as the iron, and the two liquid products may then be poured together. Or the iron may be introduced

into the liquid calcium-silicon-alloy by submerging iron-wire or rods in the liquid calcium-silicon-alloy until they are dissolved, the wire or rods being cold or red-hot.

There may be employed widely different 60 proportions of the calcium-silicon-alloy and of iron, but a good result is obtained by employing 1 kilogram of calcium-silicon-alloy and 1 to 2 kilograms of iron.

If less iron is taken than calcium-silicon-alloy, it will no longer be easy to separate the layers, the alloy containing less calcium and in consequence being of a higher specific gravity. If twice as much iron as calcium-silicon-alloy is employed or still more, an 70 alloy will be formed, containing very much calcium, but the alloy will partly remain in the slag. If, for example, 4 kilograms of calcium-silicon-alloy are melted together with 4 kilograms of iron, an alloy is obtained, containing about 64.5 per cent. of calcium, 23 per cent. of silicon and 12.5 per cent. of iron, the proportion of the calcium as compared with that of the silicon being about 74 to 26. If, on the contrary, 4 kilograms of calcium-silicon-alloy are melted together with 7 kilograms of iron, an alloy is obtained containing 53.2 per cent. of calcium, 36.9 per cent. of silicon, and 9.9 per cent. of iron. In this alloy the proportion 80 of the calcium as compared with that of the silicon is nearly 60 to 40. During this process of melting, besides the calcium-silicon-alloy, a ferro-silicon will be formed which contains more or less silicon according to the 90 amount of iron added.

In the same way as described above for the calcium-silicon-alloys, the alloys of the other alkaline earth metals with silicon may be enriched by melting them together with 95 iron.

It is to be noted that the reaction above described is also to be made use of, if, besides calcium, other active metals, as for instance aluminium, magnesium, are present 100 in the alloy, as well as other inactive metals which will form an alloy with calcium-silicon, as for instance copper, nickel, manganese etc.

What we claim is:

1. A process of increasing the amount of alkaline earth metal in alloys of silicon with alkaline earth metals by melting same with iron.
2. A process of increasing the amount of 110

calcium in alloys of silicon with calcium by melting same with iron.

3. A process of increasing the amount of alkaline earth metal in alloys of a metal which reacts chemically with alkaline earth metals, consisting in melting said alloy with iron.

4. A process of increasing the amount of calcium in alloys of a metal which reacts chemically with calcium, consisting in melting said alloy with iron.

5. A process of increasing the amount of calcium in alloys of calcium-silicon with other metals by melting same with iron.

15 6. A process of manufacturing alloys of silicon and an alkaline earth metal with a high percentage of the alkaline earth metal consisting in heating silicon together with a dissociable compound of the alkaline earth metal containing oxygen, removing the slag

formed by this reaction and melting the alloy of silicon and the alkaline earth metal thus produced with iron.

7. A process for manufacturing alloys of silicon and calcium with a high percentage 25 of calcium, consisting in heating silicon together with lime, removing the slag formed by this reaction and melting the alloy of silicon and calcium thus produced with iron.

8. As a new product, an alloy free from 30 carbon and containing calcium and silicon, the content of calcium being up to 60 and more per cent.

In testimony whereof we affix our signatures in presence of two witnesses.

HANS GOLDSCHMIDT.  
OTTO WEIL.

Witnesses:

PETER LIEBER,  
WILHELM FLASCHE.